

M. CHEW,  
METHOD OF PRODUCING FIBER BOARD,  
APPLICATION FILED OCT. 23, 1920.

1,423,083.

Patented July 18, 1922.



INVENTOR  
MANLEY CHEW.  
BY *Manley Chew* ATTYS.

# UNITED STATES PATENT OFFICE.

MANLEY CHEW, OF MIDLAND, ONTARIO, CANADA.

## METHOD OF PRODUCING FIBER BOARD.

1,423,083.

Specification of Letters Patent. Patented July 18, 1922.

Application filed October 23, 1920. Serial No. 419,051.

To all whom it may concern:

Be it known that I, MANLEY CHEW, of the town of Midland, in the county of Simcoe, Province of Ontario, Canada, have invented 5 certain new and useful Improvements in the Methods of Producing Fiber Board, of which the following is the specification.

My invention relates to certain new and useful improvements in the method of producing fiber board and particularly that 10 class of fiber board made from the chip waste of saw mills.

One object of my invention is to produce a board of this class which will be strong, 15 stiff, not liable to check or warp nor be effected by dampness or water.

A further object is to make the board durable, and to a large extent fire proof and capable of being utilized as a substitute for 20 plaster and the like in the interior finishing of a house.

My method consists in subjecting the chip waste to moisture and heat, or shortly steam, to cook the same, floating this waste and 25 beating it in such floated condition to a fibrous, watery, pulpy mass, with the fibers separated but unbroken, and practically shredded, then agitating the mass to keep 30 it in a proper consistency and carrying it in such consistency in a stream over obstructions whereby the mass is freed from foreign matter, and then precipitating or projecting the pulp in a flat filmy state into the press where the water is expressed and the 35 fiber board is finally formed, then drying and waterproofing the board.

To carry out my method I employ the following apparatus and method which I shall now describe.

40 The drawing represents the apparatus for carrying out my method.

1 is a container of any convenient size having steam pipes 2 contained in the bottom thereof. This container 1 is filled with 45 chip waste by a suitable conveyer such as is frequently used in saw mills, then water is introduced into the waste, and also preferably a powdered talc, soda ash or ground asbestos. The heat applied to the steam 50 pipes serves to convert the water into steam, which permeates the mass of waste.

The mass of waste is cooked from ten to 55 twenty-four hours depending upon the nature thereof. The steam of course passes up through the waste and softens and renders

it pliable and workable. Water is then introduced into the mass and it is then fed by any suitable means to a hopper 3 whence it is conveyed by an endless chain of buckets 4 to a hopper 5 at the top of a beater 6, or 60 series of beaters. The beater I use is the Claflin beater, although other forms of beaters may be employed.

The water introduced into the mass more or less floats the waste and converts it into 65 a rough pulplike watery condition. In the beaters the mass is so treated that the fibers are separated into very fine strands, shredded yet pulplike in form.

From the beater 6 the pulp is passed by 70 a spout 7 to a spout 8 which conveys it into the cylindrical screening machine 9, and into the cylindrical mesh screen 10 thereof. The pulp which passes through the screen 10 is conveyed by means of a pipe 11 to a receptacle 12. The pulp which does not pass through the screen 10, that is, the tailings, pass through the pipe 13 to a ball or roller mill 14 where it is rendered sufficiently fine 75 to be fed by the pipe 15 to the feed pipe 11. Instead of the beater 6, a ball or roller mill 80 may be advantageously substituted.

At this point I introduce a suitable hair or fiber, animal, vegetable or mineral, such as horse hair, shredded flax, hemp or jute or 85 asbestos. 16 is a cylindrical woven wire screen against which the pulp in the receptacle 12 impinges and 17 is a felt roll by which the pulp is rolled and carried off from the cylindrical screen in the form of long 90 strips of fine shredded pulp. Water is again introduced by the pipes 18 and 19 to cause a free flow of the pulp on to and down the chute 20 into the vat 21.

From the vat 21 a pipe 22 extends to the 95 pump 23 whereby the pulp is elevated and pumped by a pipe 24 into the agitating tank 25 which contains a series of rotary agitators 26 of any desired form such as shown in the drawing with paddles 27.

100 By means of the rotary agitators the pulp is kept at a proper and uniform consistency in the agitating tank or vat 25. From the agitating tank the pulp is carried by means of a pipe 27, pump 28, and pipe 29 into a 105 boxlike receptacle 30 having an intermediate bottom 30. The pulp passes in a stream, in the course indicated by arrow, being interrupted in its flow by slats 31 on the intermediate bottom and slats 32 on the actual 110

bottom. These slats form obstructions so as to catch any heavy foreign matter such as metal.

After the stream passes over the slats 5 the pulpy mass passes along and is precipitated or projected along down a flat chute of substantially a width corresponding to the length of the fiber board. The pulp is fed at such a speed as will induce 10 the filmy mass of pulp to feed over the entire width of the chute in its passage to the press 33 which is preferably a hydraulic one.

In the press the water is expressed from 15 the pulp, and is formed up into a solid board.

From the press the boards are stacked into kilns and dried.

After being thoroughly dried they are treated with a waterproofing liquid or com- 20 position.

I preferably treat the pulp in its passage through the apparatus with a suitable mineral binder. This may consist of powdered talc or a combination of powdered talc and 25 ground asbestos or soda ash.

In describing my method I desire it to be understood, however, that I do not wish to limit myself to the exact steps described as various changes may be made therein with- 30 out departing from the spirit of my invention.

What I claim as my invention is:

1. The method of manufacturing fiber board from chip waste consisting of steam 35 cooking the waste, then introducing water into the mass, then beating the water permeated mass, then screening it, then agitating it and then feeding the mass now reduced to pulp in a flat stream to the press, 40 then expressing the water therefrom and pressing the pulp into board form.

2. The method of manufacturing fiber board from chip waste consisting of steam cooking the waste, then introducing water 45 and a mineral binder into the mass, then

beating the water permeated mass, then screening it, then agitating it and then feeding the mass now reduced to pulp in a flat stream to the press, then expressing the water therefrom and pressing the pulp into 50 board form.

3. The method of manufacturing fiber board from chip waste consisting of steam cooking the waste, then introducing water into the mass, then beating the water permeated mass, then screening it, then rolling 55 the fibrous mass so that the fibers are more or less drawn out longitudinally, then precipitating this mass into a tank, then carrying it forward and agitating it and then feeding the mass now reduced to pulp in a flat stream to the press, then expressing the water therefrom and pressing the pulp into board form.

4. The method of manufacturing fiber 65 board from chip waste consisting of steam cooking the waste, then introducing water into the mass, then beating the water permeated mass, then screening it, then introducing a hair like binder, then rolling the 70 fibrous mass so that the fibers are more or less drawn out longitudinally, then precipitating this mass into a tank, then carrying it forward and agitating it and then feeding the mass now reduced to pulp in a flat 75 stream to the press, then expressing the water therefrom and pressing the pulp into board form.

5. The method of manufacturing fiber board from chip waste consisting of steam 80 cooking the waste, then introducing water into the mass, then beating the water permeated mass, then screening it, then agitating it and then feeding the mass now reduced to pulp in a flat obstructed stream 85 to the press, then expressing the water therefrom and pressing the pulp into board form.

MANLEY CHEW.